

## UNITED STATES PATENT OFFICE

2,272,777

## CADMIUM COATING

Georg Reuter, Markranstadt, near Leipzig,  
Germany

No Drawing. Application December 20, 1939, Serial No. 310,145. In Germany April 27, 1937

9 Claims. (CL. 91—68.3)

This invention relates to the deposition of coatings of cadmium without application of an outside source of current, by way of aqueous solutions of cadmium salts.

The process of depositing e. g. silver, copper or tin as metal coatings in a simple and economical manner according to the so-called immersion or hot bath process, without application of any outside source of electric current, is well known. It is also possible to produce nickel and brass deposits in the same manner. Great difficulties have been encountered, however, in the deposition of zinc or cadmium from aqueous solutions without application of any outside source of electric current. It has been suggested to produce metal coatings of cadmium on aluminum by dipping cleaned parts of aluminum into a solution of complex cadmium-cyanide previously heated to 60° C. This, however, yields only a very thin coating which does not offer any efficient protection. It has further been suggested to produce metal deposits on iron by boiling with a mixed solution of cadmium salt and tin-salt. It has been found, however, that by means of such a solution the deposition of pure cadmium is not possible.

It is the object of the present invention to provide a system of depositing adherent coatings of cadmium upon other metals, without application of any outside source of electric current, from aqueous solutions of cadmium salts, i. e., of at least the same thickness, as is possible with silver or tin. According to the invention, the articles to be coated are treated in potassium cyanide solutions or alkali solutions of cadmium-salt which show an excess of free alkali cyanides or caustic alkali many times that of the dissolved cadmium metal. The cadmium coating may be deposited, e. g., on copper, brass, copper plated or brass plated iron, but also directly on iron. The coating is most easily formed in an adherent and brilliant form on surfaces or alloys like brass.

Cyanogen-cadmium baths are well known in galvano-technics, which for attaining bright and brilliant coatings by application of electric current contain a certain excess of caustic soda and cyanide of sodium. Such baths, however, cannot be used in connection with a hot treatment without electric current. Moreover, it has been found that the hot baths to suit the different procedure, must also be prepared in an entirely different way. The current would deposit cadmium metal from pure solutions of cyanide of cadmium, but, when applying a hot bath, a deposition of pure cadmium will be obtained only

if the bath contains large excessive amounts of alkali cyanides or caustic alkali in relation to the cadmium dissolved.

According to the invention the production of 5 cadmium coatings directly upon blank iron, can be attained by boiling the articles in very hot baths at temperatures exceeding 100° C. Such temperatures according to the invention, can be made possible by a considerable admixture of 10 soda or by a heavy increase of the amount of free, excessive caustic alkali in the contents of the bath. Some alkali cyanide can also be provided, if available. Provided that sufficiently high temperatures are attained, the direct coating of 15 blank iron with cadmium does not offer any difficulties. The cadmium is deposited in an adherent form, which can be easily polished and offers good protection against corrosion. With certain sorts of iron the coating with cadmium is facilitated by a previous short pickling treatment with mineral acids or similar acids.

For the deposition of cadmium coatings on articles made of brass, according to the invention, the bath can be composed as follows:

About 4 grams cadmium in the form of its oxide, chloride, carbonate or in some other form of salt. About 70 to 150 grams alkali cyanide, 1000 grams water, temperature: 40 to 70° C.

For depositing cadmium coatings on blank 20 iron, the following composition for the bath would be suitable:

About 5 to 8 grams cadmium in the form of its oxide or salts, about 1200 to 1400 grams caustic soda or caustic potash, 1000 grams water, with 25 or without the addition of some alkali cyanide, temperature: about 125° C.

The method of the present invention has been described in detail with reference to specific embodiments. It is to be understood, however, that 30 the invention is not limited by such specific reference but is broader in scope and capable of other embodiments than those specifically described.

I claim:

- 45 1. A process of producing adherent coatings of cadmium to be deposited on a metal of the group consisting of copper, brass, iron, copper-plated iron, and brass plated iron, without the application of an outside source of electric current, by means of a hot bath treatment, in which the articles to be coated are treated in hot aqueous alkali cadmium salt solutions which contain an excess of free caustic alkali many times by weight that of the dissolved cadmium metal.
- 50 2. A process of producing adherent coatings

of cadmium on a metal of the group consisting of copper, brass, iron, copper-plated iron, and brass plated iron, without application of an outside source of electric current, by means of a hot bath treatment, in which the articles to be coated are treated in hot aqueous alkali cadmium salt solutions which contain an excess of free alkali cyanides many times by weight that of the dissolved cadmium metal.

3. A process for the production of adherent coatings of cadmium on a metal of the group consisting of copper, brass, iron, copper-plated iron, and brass plated iron, without application of an outside source of electric current, by means of a hot bath treatment, in which the articles to be coated are treated in hot aqueous potassium cyanide solutions of cadmium salt which contain an excess of free alkali cyanides many times by weight that of the dissolved cadmium metal.

4. A process for the production of adherent coatings of cadmium on a metal of the group consisting of copper, brass, iron, copper-plated iron, and brass plated iron, without application of an outside source of electric current, by means of a hot bath treatment, in which the articles to be coated are treated in hot aqueous potassium cyanide solutions of cadmium salt which contain an excess of free caustic alkali many times by weight that of the dissolved cadmium metal.

5. A process for the production of adherent coatings of cadmium on iron, without application of an outside source of electric current, by means of a boiling treatment, in which the articles to be coated are treated in aqueous solutions of the group consisting of potassium cyanide solutions and alkali solutions of cadmium salts which contain an excess of alkali of the group consisting of alkali cyanides and caustic alkali many times by weight that of the dissolved cadmium metal and in which the boiling treatment

is carried out at a temperature exceeding 100° C.

6. A process for the production of adherent coatings of cadmium on iron without application of an outside source of electric current, by means of a boiling treatment, in which the articles to be coated are treated in aqueous cadmium salt solutions of the group consisting of potassium cyanide solutions and alkali solutions of cadmium salts which contain an excess of alkali of the group consisting of alkali cyanides and caustic alkali many times by weight that of the dissolved cadmium metal and in which the boiling treatment is carried out at a temperature exceeding 100° C., this temperature being made possible by a heavy addition to the bath of an alkali of the group consisting of soda and caustic alkali.

7. A process for the production of an adherent coating of cadmium on brass without application of an outside source of electric current, by means of a hot bath treatment in which the articles to be coated are treated in a solution of approximately four parts by weight of a substance selected from the group consisting of the oxide and the salts of cadmium, between 70 and 150 parts by weight of an alkali cyanide in 1000 parts by weight of water at a temperature between 40 to 70° C.

8. A process for the production of an adherent coating of cadmium on blank iron without application of an outside source of electric current by means of a boiling treatment, in which the articles to be coated are treated in a bath containing between 5 and 8 parts by weight of a substance selected from the group consisting of the oxide and the salts of cadmium, between 1200 and 1400 parts by weight of a caustic alkali, and about 1000 parts by weight of water, at a temperature of about 125° C.

9. A process as claimed in claim 8, wherein some alkali cyanide is added to the bath.

GEORG REUTER.